

## 1

3,579,289

**ACID SALT FORM OF DEAE CELLULOSIC FABRIC PROVIDING BUILT-IN CATALYSIS FOR THE REACTION WITH AMINOPLASTS**

Donald M. Soignet, Metairie, and Ruth R. Benerito, New Orleans, La., assignors to the United States of America as represented by the Secretary of Agriculture  
 No Drawing. Filed Jan. 16, 1970, Ser. No. 3,514  
 Int. Cl. C08b 11/20; D06m 13/40, 13/54  
 U.S. Cl. 8—116.3

7 Claims

**ABSTRACT OF THE DISCLOSURE**

Diethylaminoethylated cellulosic fibers, the diethylaminoethyl groups of which are in an acid salt form, provide a built-in catalyst for the reaction of said fibers with methyloolated nitrogen containing cross-linking agents with which said fibers are contacted.

A nonexclusive, irrevocable, royalty-free license in the invention herein described, throughout the world for all purposes of the United States Government with the power to grant sublicenses for such purposes, is hereby granted to the Government of the United States of America.

It is well known in the art that the cellulose hydroxyls will react with substituted cyclic ureas in the presence of a catalyst. These catalysts, which are added to the reagent solution, are usually ammonium salts (Cooke, J. F., Roth, P. B., Salsbury, J. M., Switlyk, G., and van Loo, W. J., Tex. Res. J. 27, 150-165, 1957), or metal salts (Marsh, J. T., Tex. Mfr., 86, 113, 1960). Once, however, the solution of catalyst and reagent are padded onto the fabric and the fabric dried at low temperatures (below 70° C.), the reaction between the reagent and the cellulose will proceed rapidly on the application of heat or at a somewhat slower rate at room temperature. This negates the possibility of padding the reagent and catalyst on a fabric and then storing it for long periods of time before curing.

The process described in this invention differs from the art in that the catalyst is incorporated first as an integral part of the cellulosic material and thus need not be added to the reagent solution. The fabric padded in this manner will not react with the reagent solution until

## 2

curing temperatures are attained. It is then possible to store the reagent on the fabric without fear of reaction. The reaction can be initiated when curing temperatures are reached.

In carrying out the preferred process of this invention, cellulosic fabric is treated with a 20% aqueous solution of 2-chloroethyldiethylamine hydrochloride and cured in 8% sodium hydroxide at 95° C. according to the method of Soignet and Benerito (Tex. Res. J., 37, 1001-1003, 1967). The diethylaminoethylated (DEAE) cellulose thus produced is soaked in 0.1 N sodium hydroxide to convert it to the base form. This fabric is then converted to the desired acid salt by soaking in a 0.5 N solution of the corresponding acid. Unbound acid is then washed out and the fabric is then padded to a 100% wet pickup with an aqueous solution of the desired substituted cyclic urea and dried at 60° C. for about 7 minutes. The fabric can now be cured at elevated temperatures or set aside and cured at some later date.

Cellulosic materials such as cotton, rayon, ramie, jute, and flax and in the form of fiber, yarn, fabric or powder may be used in the process of this invention. The degree of crosslinking in the ion exchange powdered material diethylaminoethyl cellulose can also be increased by the process of this invention.

The following examples illustrate but do not limit the scope of this invention. Breaking strength tests were carried out according to the ASTM Method D1682-64. Condition wrinkle recovery measured were determined according to the ASTM D1295-67 method and the wet recovery measurements according to the method described by Fujimoto, R. A., et al. (American Dyestuff Repr., 52, 329, 1963).

**EXAMPLE 1**

Cotton printcloth, treated to contain 0.50% nitrogen in the form of diethylaminoethyl cellulose, soaked in various acids to insure that the amine was in the acid form, washed free of unbound acid, was padded with a 10% aqueous solution of dimethylolethylene urea [1,3-bis(hydroxymethyl)-2-imidazolidinone]. The fabric was dried at 60° C. for 7 minutes and cured at 160° C. for 3 minutes. After curing the fabric was washed free of non-bound reagent and air dried. The following table summarizes results of properties measured in cured fabric.

| Associated acid                | Nitrogen added, weight, percent | Formaldehyde weight, percent | Wrinkle recovery (W plus F), degrees |                          | Breaking strength, pounds | Elongation, percent | M.S. <sup>2</sup> |
|--------------------------------|---------------------------------|------------------------------|--------------------------------------|--------------------------|---------------------------|---------------------|-------------------|
|                                |                                 |                              | Wet <sup>1</sup>                     | Conditioned <sup>1</sup> |                           |                     |                   |
| Acetic                         | 2.76                            | 2.36                         | 222 (56)                             | 280 (88)                 | 29                        | 9                   | 0.16              |
| Formic                         | 2.43                            | 2.95                         | 236 (77)                             | 279 (89)                 | 28                        | 8                   | 0.14              |
| Citric                         | 3.42                            | 2.01                         | 247 (63)                             | 304 (120)                | 28                        | 8                   | 0.20              |
| HCl                            | 2.14                            | 2.60                         | 238 (74)                             | 288 (74)                 | 28                        | 8                   | 0.13              |
| H <sub>2</sub>                 | 2.08                            | 3.67                         | 231 (64)                             | 281 (84)                 | 27                        | 8                   | 0.12              |
| H <sub>2</sub> F               | 1.90                            | 3.15                         | 216 (48)                             | 277 (73)                 | 29                        | 8                   | 0.11              |
| H <sub>2</sub> SO <sub>4</sub> | 1.89                            | 2.97                         | 200 (33)                             | 271 (75)                 | 28                        | 9                   | 0.11              |
| H <sub>3</sub> PO <sub>4</sub> | 1.58                            | 2.67                         | 218 (47)                             | 289 (85)                 | 29                        | 9                   | 0.09              |
| HClO <sub>4</sub>              | 1.89                            | 3.25                         | 241 (71)                             | 280 (75)                 | 29                        | 8                   | 0.11              |

<sup>1</sup> Bracketed numbers represent the increase in wrinkle recovery with respect to each control fabric (DEAE-HX).

<sup>2</sup> M.S. represents molar substitution based on nitrogen added to the fabric by DME U treatment and based on one DME U unit per crosslink.

**3**  
**EXAMPLE 2**

Diethylaminoethyl cotton of 0.9% nitrogen in the hydrochloride form is padded with a 10% aqueous solution of dimethylolethylene urea; dried at 60° C. for 7 minutes and cured at various temperatures for 3 minutes. Results of treated fabrics shown below.

| Cure temperature, °C.: | Nitrogen added, weight, percent | Formaldehyde weight, percent | Wrinkle recovery (W plus F), degrees |             |                           | Elongation, percent | M.S. <sup>1</sup> |
|------------------------|---------------------------------|------------------------------|--------------------------------------|-------------|---------------------------|---------------------|-------------------|
|                        |                                 |                              | Wet                                  | Conditioned | Breaking strength, pounds |                     |                   |
| 100                    | 0.47                            | 0.89                         | 196                                  | 217         | 41                        | 14                  | .025              |
| 110                    | 0.84                            | 1.67                         | 206                                  | 234         | 38                        | 14                  | .050              |
| 120                    | 1.23                            | 2.47                         | 231                                  | 254         | 33                        | 12                  | .070              |
| 130                    | 1.66                            | 2.57                         | 234                                  | 280         | 28                        | 14                  | .095              |
| 140                    | 1.67                            | 3.26                         | 252                                  | 273         | 27                        | 13                  | .095              |
| 150                    | 1.75                            | 3.29                         | 267                                  | 287         | 25                        | 13                  | .100              |
| 160                    | 1.79                            | 2.69                         | 266                                  | 297         | 21                        | 13                  | .105              |
| 170                    | 1.67                            | 2.91                         | 267                                  | 293         | 22                        | 16                  | .095              |
| DEAE control           | 0.94                            | -----                        | 194                                  | 165         | 37                        | 22                  | -----             |

<sup>1</sup> M.S. represents molar substitution based on nitrogen added to fabric by DMEU treatment and based on one DMEU unit per crosslink.

**EXAMPLE 3**

Diethylaminoethyl cotton of 0.5% nitrogen in the hydrochloride form is padded with various concentrations of dimethylolethyleneurea, dried 7 minutes at 60° C. and cured at 160° C. for 3 minutes. Results obtained are listed below.

| DMEU concentration weight, percent: | Nitrogen added, weight, percent | Formaldehyde weight, percent | Wrinkle recovery (W plus F), degrees |             |       | M.S. <sup>1</sup> |
|-------------------------------------|---------------------------------|------------------------------|--------------------------------------|-------------|-------|-------------------|
|                                     |                                 |                              | Wet                                  | Conditioned |       |                   |
| 1                                   | 0.18                            | 0.37                         | 204                                  | 234         | 0.01  | 35                |
| 4                                   | 0.69                            | 1.26                         | 246                                  | 270         | 0.04  |                   |
| 5                                   | 0.83                            | 1.55                         | 247                                  | 275         | 0.05  |                   |
| 6                                   | 0.97                            | 1.78                         | 248                                  | 281         | 0.05  |                   |
| 8                                   | 1.35                            | 2.45                         | 257                                  | 283         | 0.08  |                   |
| 10                                  | 1.41                            | 2.81                         | 256                                  | 272         | 0.08  |                   |
| DEAE control                        | 0.49                            | -----                        | 189                                  | 183         | ----- | 40                |

<sup>1</sup> M.S. based on nitrogen added to fabric by DMEU treatment and based on one DMEU unit per crosslink.

Diethylaminoethyl cotton of varying nitrogen content and in the hydrochloride form is padded with a 10% aqueous solution of dimethylolethylene urea, dried 60° C. for 7 minutes, and cured at 160° C. for 3 minutes. Results obtained are summarized below.

| Original nitrogen content, weight, percent | Nitrogen added, weight, percent | Formaldehyde weight, percent | Wrinkle recovery (W plus F), degrees |             |      | M.S. <sup>1</sup> |
|--------------------------------------------|---------------------------------|------------------------------|--------------------------------------|-------------|------|-------------------|
|                                            |                                 |                              | Wet                                  | Conditioned |      |                   |
| 0.06                                       | 1.26                            | 1.83                         | 216                                  | 212         | 0.07 |                   |
| 0.10                                       | 1.28                            | 1.87                         | 221                                  | 239         | 0.07 |                   |
| 0.15                                       | 1.07                            | 1.74                         | 226                                  | 241         | 0.06 |                   |
| 0.17                                       | 1.17                            | 1.88                         | 228                                  | 256         | 0.07 |                   |
| 0.20                                       | 1.26                            | 2.03                         | 229                                  | 260         | 0.07 |                   |
| 0.49                                       | 1.41                            | 2.81                         | 256                                  | 272         | 0.08 |                   |
| 0.94                                       | 1.79                            | 2.69                         | 266                                  | 297         | 0.10 |                   |

<sup>1</sup> M.S. is molar substitution based on nitrogen added to fabric by DMEU treatment and based on one DMEU unit per crosslink.

**EXAMPLE 5**

Diethylaminoethyl cottons containing 0.5% nitrogen in the hydrochloride form are treated with 8% dimethylolethylene urea in various solvents, dried at 60° C. for 7 minutes, and cured at 160° C. for 3 minutes.

| Solvent                                         | Wrinkle recovery |             |       | Molar substitutes |
|-------------------------------------------------|------------------|-------------|-------|-------------------|
|                                                 | Wet              | Conditioned |       |                   |
| H <sub>2</sub> O                                | 260              | 288         | ----- | .08               |
| DMF                                             | 245              | 278         | ----- | .08               |
| 90% DMF plus 10% H <sub>2</sub> O               | 250              | 270         | ----- | .08               |
| 90% dioxane plus 10% H <sub>2</sub> O           | 266              | 282         | ----- | .09               |
| 90% EtOH plus 10% H <sub>2</sub> O              | 268              | 285         | ----- | .09               |
| 90% THF plus 10% H <sub>2</sub> O               | 270              | 290         | ----- | .125              |
| 98% methylene chloride plus 2% H <sub>2</sub> O | 245              | 282         | ----- | .05               |
| 1,3-dichloro-2-propanol                         | 258              | 290         | ----- | .07               |
| 1-chloro-2-propanol                             | 250              | 283         | ----- | .04               |

**4**  
**EXAMPLE 6**

Diethylaminoethyl cottons of 0.9% nitrogen in the hydrochloride form are padded with 10% aqueous solutions of the following reagents: (1) dimethylolethyleneurea (DMEU), 1,3-bis(hydroxymethyl)-2-imidazolinone; (2) dimethylolpropyleneurea (DMPU), 1,3-bis(hy-

droxymethyl)-2(IH)-tetrahydropyrimidinone; (3) dihydroxyethyleneurea (DHEU), 4,5-dihydroxy-2-imidazolinone, and (4) dimethyldihydroxyethyleneurea (DMDHEU), 1,3-bisdimethyl-4,5-dihydroxy-2-imidazolidinone, (5) dimethyloldihydroxyethyleneurea (DMDHEU), 1,3-bis(hydroxymethyl) - 4,5 - dihydroxy-2-imidazolidinone. Each is dried at 60° C. for 7 minutes and cured at 160° C. for 5 minutes. Results obtained are summarized below.

| Reagent | Wrinkle recovery |     | Molar substitution |
|---------|------------------|-----|--------------------|
|         | Wet              | Dry |                    |
| DMEU    | 275              | 285 | .10                |
| DMPU    | 265              | 295 | .10                |
| DHEU    | 272              | 237 | .09                |
| DMDHEU  | 270              | 233 | .08                |
| DMDHEU  | 274              | 242 | .04                |

**EXAMPLE 7**

Diethylaminoethyl cotton of 0.2% nitrogen in the hydrochloride form is padded to 100% wet pickup with a 10% aqueous dimethylolethyleneurea solution, dried at 60° for 7 minutes. The fabric is allowed to stand at room temperature in this condition until ready for curing. At various intervals portions of fabric are removed. They are tested for nitrogen and crease recovery. At the same time, another portion is cured at 160° C. for 3 minutes. Results are tabulated below.

| Days delay: | Percent nitrogen added— |            | Wrinkle recovery |     |     |  |
|-------------|-------------------------|------------|------------------|-----|-----|--|
|             | Before cure             | After cure | Before cure      |     |     |  |
|             |                         |            | Wet              | Dry |     |  |
| 0           | 0.00                    | 1.55       | 175              | 190 | 275 |  |
| 8           | 0.02                    | 1.52       | 175              | 185 | 285 |  |
| 16          | 0.04                    | 1.45       | 160              | 187 | 240 |  |
| 22          | 0.10                    | 1.45       | 180              | 186 | 275 |  |

**EXAMPLE 8**

DEAE cotton in the hydrochloride form containing 0.77% N is padded twice to 100% wet pickup with an 8% aqueous solution of dimethyloldihydroxyethyleneurea (DMDHEU). It is dried at 60° C. for 7 minutes. The fabric is then allowed to remain under room conditions until curing is desired. A portion is removed, washed in cold then hot tap H<sub>2</sub>O and ironed dry. At the same time, another portion is removed and cured at 160° C. for 3 minutes and then washed in hot tap H<sub>2</sub>O and ironed dry. Results obtained after varying delay times are tabulated in the following table:

| Percent<br>N added | Before cure—                |              |     |                    | After cure—                 |              |     |     |
|--------------------|-----------------------------|--------------|-----|--------------------|-----------------------------|--------------|-----|-----|
|                    | Percent<br>formal-<br>dehyd | Crease angle |     | Percent<br>N added | Percent<br>formal-<br>dehyd | Crease angle |     |     |
|                    |                             | Wet          | Dry |                    |                             | Wet          | Dry |     |
| Delay (days):      |                             |              |     |                    |                             |              |     |     |
| 0                  | 0                           | .02          | 197 | 164                | .77                         | 1.03         | 281 | 274 |
| 14                 | .07                         | .02          | 192 | 192                | .77                         | 1.07         | 269 | 284 |
| 28                 | .03                         | .02          | 173 | 170                | .80                         | 1.20         | 263 | 288 |

## EXAMPLE 9

DEAE cotton in the hydrochloride form containing 0.77% N is padded twice to 100% wet pickup with a 10% aqueous solution of dimethylolmethylcarbamate. The fabric is dried at 60° C. for 7 minutes. The fabric is then allowed to remain under room conditions until curing is desired. At that time a portion is removed and washed in cold then hot tap H<sub>2</sub>O and ironed dry. At the same time another portion is removed and cured at 160° C. for 3 minutes. It is then washed in hot tap H<sub>2</sub>O and ironed dry. Results obtained after varying delay times are tabulated below.

| Percent<br>N added | Before cure—                |              |     |                    | After cure—                 |              |     |     |
|--------------------|-----------------------------|--------------|-----|--------------------|-----------------------------|--------------|-----|-----|
|                    | Percent<br>formal-<br>dehyd | Crease angle |     | Percent<br>N added | Percent<br>formal-<br>dehyd | Crease angle |     |     |
|                    |                             | Wet          | Dry |                    |                             | Wet          | Dry |     |
| Delay (days):      |                             |              |     |                    |                             |              |     |     |
| 0                  | 0                           | .04          | 187 | 165                | .37                         | 1.00         | 227 | 223 |
| 14                 | .04                         | .02          | 172 | 180                | .36                         | .92          | 205 | 236 |
| 28                 | .01                         | .02          | 176 | 186                | .36                         | 1.12         | 208 | 249 |

## We claim:

1. A process for treating a fabric which fabric can be stored before curing and possesses increased wrinkle recovery after curing which process comprises:

(a) treating a fabric composed of cellulosic fibers which have been diethylaminoethylated and which have been treated with an acid to convert the diethylaminoethyl groups thereof to the acid salt form with a solution of an N-methylol type compound selected from the group consisting of dimethylolethyleneurea, dimethylolpropyleneurea, dihydroxyethyleneurea, dimethylolhydroxyethyleneurea, dimethyloldihydroxyethyleneurea, and dimethylolmethyl carbamate;

(b) drying the treated fabric and (c) curing the dried fabric at an elevated temperature.

2. The process of claim 1 wherein the N-methylol type compound is dimethylolethyleneurea.

3. The process of claim 1 wherein the N-methylol type compound is dimethylolpropyleneurea.

4. The process of claim 1 wherein the N-methylol type compound is dihydroxyethyleneurea.

5. The process of claim 1 wherein the N-methylol type compound is dimethylolhydroxyethyleneurea.

6. The process of claim 1 wherein the N-methylol type compound is dimethyloldihydroxyethyleneurea.

7. The process of claim 1 wherein the N-methylol type compound is dimethylolmethyl carbamate.

## References Cited

## UNITED STATES PATENTS

2,584,114 2/1952 Daul et al. 8—116.3

40 GEORGE F. LESMES, Primary Examiner

J. CANNON, Assistant Examiner

## U.S. CL. X.R.

45 8—116.2; 260—232